

April 9, 1946.

J. B. NILES

2,398,110

APPARATUS FOR ELECTROLYTIC TREATMENT

Filed Oct. 10, 1941

*Fig. 1.*



*Fig. 2.*



Inventor:  
Joseph B. Niles.  
By Ehrmann, Wiles, Davies & Hirsch.  
Atty's.

## UNITED STATES PATENT OFFICE

2,398,110

APPARATUS FOR ELECTROLYTIC  
TREATMENT

Joseph B. Niles, Chicago, Ill., assignor to  
Thomas J. Dee & Co., a corporation of Illinois

Application October 10, 1941, Serial No. 414,509

5 Claims. (Cl. 204—56)

This invention relates to an improved lead-silver alloy for use in connection with apparatus for electroplating, anodizing, or the like.

The primary object of the invention is to provide an improved alloy of lead and silver which will have long life in spite of being subjected to electrolytes containing chromic acid, sulphuric acid, or other highly corrosive liquids. The alloy is of particular use for making linings, heating coils, temperature indicators, and temperature regulating instruments employing fully immersed bulbs containing expansive liquids or thermocouples. Bulbs to be protected when immersed in chromic acid solutions may have an outer covering of the alloy of suitable thickness.

A further object of the invention is to provide an alloy which may be used as a cathode or anode in an electrolyte which in use will form an oxide of high electrical conductivity and will not seriously interfere with the maintenance of current densities necessary to efficient electrolytic operations.

Heretofore, it has been common practice to use a lead-antimony material and it has been necessary to frequently clean the exposed surfaces because the chromic acid solution quickly forms compounds such as lead-chromate.

In chromium plating work, because of the low electrical conductivity of the electrolyte, high amperages are ordinarily employed. This current value may range from 115 amperes per square foot area of articles being plated to 800 amperes per square foot, and there is produced an objectionable amount of compounds on the anode surface. An analysis of these compounds shows them to be a mixture of compounds such as lead dioxide ( $PbO_2$ ), lead suboxide ( $Pb_2O$ ), and lead chromate ( $PbCrO_4$ ). All of these compounds, because of their low electrical conductivity values, seriously interfere with the maintenance of current densities necessary to continuous chromium deposition. Compounds that interfere with the flow of the electrical current must be removed at frequent intervals to restore the anode surface to proper working efficiency. In commercial practice, it is found necessary in some cases to remove the anodes for cleaning several times a day.

These difficulties have been overcome by the present invention through the use of a lead-silver alloy. It was found that the compounds of silver formed in an electrolyte of chromic acid, when subjected to the required current densities, show excellent electrical performance, and that the

amount of current drop was directly proportionate to the amount of silver combined with lead up to a percentage of about 8% of silver present. Anodes containing upwards of 8% of silver indicated no measurable current drop during a steady current flow for the duration of an hour; this time being considerably in excess of that required in the conventional chromic acid solution used in the chromium plating of articles for decorative, or ornamental, or oxidation resistant purposes.

Silver-lead alloys containing more than 10% silver by weight and used as anodes in chromium plating work offered no appreciable advantage in this respect. However, it was found that silver-lead alloys used in this work and containing more than 12% silver by weight gave indications of silver migrating from the anode to the cathode under electrolysis, and it appeared as metallic silver codeposited with metallic chromium. Silver-lead alloys containing 12% or less silver produced no apparent silver at the cathode under electrolysis.

In a series of tests, 6 lead-silver alloys were prepared, the first having 4% silver, the second 6%, etc., up to 14%, inclusive. 6 one-gallon aqueous solutions of chromic acid were made, each containing 53 ounces of chromic acid and .53 ounces of 66° Bé. sulphuric acid. Into each of these solutions was placed one of the above mentioned alloys to serve as an anode. The surface area of each anode exposed to the chromic acid solution in all cases was 8 square inches. Also, into each of these solutions was placed a strip of chemically clean pure nickel, each having an exposed area to the chromic acid solution of 8 square inches. The nickel, of course, served as a cathode in each case and a current density of 18 amperes at 6 volts was then impressed on the surface of each lead-silver alloy anode and continued until an ampere meter employed in the electrical circuit gave indications of current drop.

In observing the electrical performance of these various compositions of lead-silver anodes in this test, it was found that those alloys with less than 8% of silver gave indications of current drop or gradual falling off of current densities as the testing progressed.

An electrode containing 9 parts of lead to 1 part of silver shows thoroughly satisfactory results in a full size commercial installation. The conventional equipment is illustrated in the accompanying drawing, in which—

Figure 1 is a plan view from above showing the open top tank and the anode and cathode

bus-bars; and Figure 2 is a sectional view, taken as indicated at line 2 of Figure 1.

In the equipment illustrated a suitable tank 3 is lined with the lead-silver alloy, as indicated at 4, so that the lining fully protects the outer shell. Cathode bus-bars 5 extend over the tank and are supported in suitable insulating brackets 6. Also, the anode bus-bars 7 extend over the tank and are supported in insulating brackets 8. The anodes 9 are formed of the lead-silver alloy and are provided at their upper ends with conventional hooks 10 to enable them to be suspended from the bus-bars. The temperature of the bath may be maintained by suitable coils (not shown) in the electrolyte or by apparatus outside of the tank 3. Preferably, the lining of the anodes and other parts of the equipment that contact the electrolyte are made of the lead-silver alloy. It will be understood that the articles to be plated will be suspended from the bus-bar 5.

The lining made up of about 9 parts lead to 1 part of silver is preferably about  $\frac{1}{8}$  of an inch thick and the seams and joints rendered liquid tight.

Although the initial cost of this lining material is more than the common lead antimony lining, the new alloy will provide a substantial saving because the tanks do not have to be taken out of operation for re-lining at such frequent intervals and the combined cost of the lead antimony alloy and labor for several re-linings is in excess of the cost of one installation of the lead-silver lining.

It will be understood that the lead-silver alloy lining may be used with any suitable backing frame such as wood, metal, or the like. If preferred, the alloy may be rolled onto a metal backing before being assembled into a tank.

In the anodic treatment of aluminum, a process whereby a coating of aluminum oxide is produced on the surface of aluminum by electrolysis, similar apparatus to that described above may be used except that the aluminum forms the anode and the lead-silver alloy the cathode, which may be either separate electrodes or the lining of the tank.

Because of the higher current pressures used

in this work (40 volts), the same difficulties are encountered when a lead-antimony alloy is used, and these difficulties are overcome by the use of the lead-silver alloy. The electrolytes used for either the anodic treatment of the aluminum or chromium plating consist of the same oxidizing reagents, namely, chromic acid and sulphuric acid. By using a lead-silver alloy consisting of 9 parts of lead to 1 part of silver as cathodes, either of the suspended immersed type or as the tank lining type, the same excellent electrical conductivity of the oxides of silver is utilized to advantage.

The foregoing detailed description has been given for clearness of understanding only, and no unnecessary limitations should be understood therefrom for some modifications will be obvious to those skilled in the art.

I claim:

20. 1. An electrode consisting essentially of 6% to 12% of silver and the balance being substantially all lead and having on a surface thereof a coating of lead chromate and silver chromate having substantially the same conductivity in a chromic acid plating bath as the underlying alloy.
25. 2. An electrode consisting essentially of 8% to 12% of silver and the balance being substantially all lead and having on a surface thereof a coating of lead chromate and silver chromate having substantially the same conductivity in a chromic acid plating bath as the underlying alloy.
30. 3. An electrode as set forth in claim 1, in which the electrode is a cathode.
35. 4. The method which comprises passing an electric current through a bath containing chromic acid in which one of the electrodes exposed to the bath has an exposed surface of lead-silver alloy containing from 6% to 12% silver, whereby a surface coating of lead-silver chromate is formed which is substantially insoluble in the solution and which does not appreciably affect the resistance of the system.
40. 5. The method as set forth in claim 4, in which the proportions of the metals are approximately 9 parts of lead to 1 part of silver.

JOSEPH B. NILES.